

Dec. 5, 1933.

W. KLUGE

1,938,431

PROCESS OF MAKING PHOTO ELECTRIC TUBES

Filed May 18, 1931



Inventor:  
Werner Kluge,  
by *Charles J.alla*  
His Attorney

## UNITED STATES PATENT OFFICE

1,938,431

PROCESS OF MAKING PHOTO-ELECTRIC  
TUBES

Werner Kluge, Berlin-Hermsdorf, Germany,  
assignor to General Electric Company, a corporation of New York

Application May 18, 1931, Serial No. 538,081,  
and in Germany May 21, 1930

## 1 Claim. (Cl. 250—27.5)

It is known to use alkali metals, and preferably potassium, for tubes operable on the photo-electric effect. When the tube is used for industrial purposes, the photo-electric electron emission of the layer of pure potassium is too small so that the said layer must be sensitized according to the process described by Elster and Geitel. Hydrogen is introduced into the tube at low pressure and a glow discharge is thereafter caused to take place for a short period between the electrodes of the tube. A layer of potassium hydride is formed for the most part and is recognizable by its blue-violet color. In the best of tubes, the photo-electric output over the light spectrum, i. e., the number of electrons released from a layer of this kind (and in relation to the wave length) for each incident monochromatic unit of light energy is shown by the curve 1 in the accompanying drawing. There is no photo-electric action above the wave length  $550\mu\mu$ , known as the red border.

Hydrides have proved to be very unstable as a photo-electric sensitive substance. They disintegrate under the action of light and are dissociated by the positive ions of the rare gases of the tube, the said gases impinging on the light-sensitive layer when the load is put on the tube. This layer evaporates when heated (about  $70^\circ$ ). For these reasons, the life of tubes of this kind is comparatively short and the defect is particularly troublesome when the tubes are used in sound film machines, in which capacity they should stand a long-period load with unvarying sensitiveness.

The subject-matter of the invention is an improved process for the manufacture of photo-electric tubes which are free from the defects mentioned in the foregoing. The principle of the invention is explained hereunder.

A portion of the inner wall of the vessel of the tube is first silvered according to a known process, for example by placing in the said vessel a solution of silver nitrate and adding a reducing solution thereto which is measured so that the silver is precipitated at the desired point on the glass wall. The tube is now connected to the pump and is exhausted while simultaneously heated to about  $370^\circ$  C. for a long period of time in order to expel gas and dampness residues liable to affect the operation of the tube detrimentally at a later stage. Dry oxygen is now admitted to a pressure of fractions of one millimetre of mercury and a pulsating glow discharge produced through the tube by applying thereto a direct-current voltage of

about 400 with the aid of a suitable series resistance. The discharge is maintained until a visible alteration in the layer of silver indicates the presence of an adsorbed layer of oxygen. After being thus treated, the layer of silver assumes a yellowish tint. The foundation layer for the alkali metal being now ready, the said metal is now distilled, through the pump connection, into the envelope preliminarily treated in this manner. The quantity of alkali metal is such that the foundation layer becomes faintly dull. If voltage is now applied to the tube, a photo-electric current may be produced by illumination.

According to the invention, the sensitiveness of the tube, especially in the infra-red region of the spectrum, may be further increased in the following manner. The tube is heated to about  $200^\circ$  C. for a few seconds, preferably by means of a large flame surrounding the whole tube and the atomic potassium vapor is adsorbed on the layer of oxygen. Particularly good results are obtained by additionally ionizing the potassium vapor within the tube. To this end, a voltage of about 100 volts is applied during the short period of time within which the tube is heated. Electrons are liberated by illumination of the cathode to produce potassium ions by collision on their way to the anode. This ionizing current may be measured by means of an ammeter disposed in the load circuit, but of course remains in existence only for a short time because the potassium vapor gradually flows back to the distilling apparatus through the pump connection. The positive alkali metal ions are adsorbed on the oxygen layer and form a highly sensitive layer. The distilling apparatus is cooled as soon as this ionizing current is detected by the ammeter and the non-ionized and non-adsorbed vapor is caused to return to the distilling apparatus by further heating the tube. The cooling action takes effect immediately behind the pump connection by introducing compressed air, whereafter the production of the light-sensitive layer is completed; the tube may now be filled with rare gas and sealed off.

The spectroscopic output of the improved photo-electric tube provided with a layer of this kind is shown by curve No. 2 in the drawing. This curve is of considerably greater amplitude in all parts of the spectrum than in the case of a layer of potassium hydride. The positive ion current of the rare gas which impinges on the light-sensitive layer when the tubes are put under load, produces no alteration in the emitting power. Also, the properties of the layer are not

altered when the latter is subjected to the action of a relatively large amount of heat. The life of the tubes is thus much longer and answers industrial requirements.

5 The sensitiveness in the red zone of the spectrum is remarkable because photo-electric action may be detected at about  $800\mu\mu$ . A tube improved in accordance with the present invention may also be used as a receiving instrument for 10 modulated infra-red waves in ultra-short wave telephony.

While I have described my invention more particularly with reference to potassium as the light-sensitive material, it is to be understood 15 that the improved process is also applicable to

alkali metals in general, including sodium, caesium and rubidium.

What I claim as new and desire to secure by Letters Patent of the United States, is:

In the manufacture of a photo-electric tube, 80 the method which comprises the following steps; coating the interior of the envelope with a foundation layer of metal, introducing oxygen into the tube, passing a glow discharge to oxidize the metal layer, admitting alkali metal into the tube, 85 heating the tube to vaporize the alkali metal and applying a voltage to the tube during the heating period to cause current to flow through the tube and to sensitize the alkali metal.

WERNER KLUGE. 90

28

95

25

100

30

105

35

110

40

115

45

120

50

125

55

130

60

135

65

140

70

145

75

150